

March 2, 1965

O. PETER ET AL

3,171,816

FABRICATION OF CARBON BODIES

Filed Nov. 29, 1960

2 Sheets-Sheet 1

FIG. 1



AMOUNT, IN % BY WEIGHT, OF AGENT ADDED FOR  
REDUCING THE SOFTENING POINTS OF THE  
BINDING PITCH

INVENTORS.  
OTTO PETER  
HELMUT RECKHARD  
BY

*Curtis, Morris & Lafford*  
ATTORNEYS

March 2, 1965

O. PETER ETAL

3,171,816

FABRICATION OF CARBON BODIES

Filed Nov. 29, 1960

2 Sheets-Sheet 2

FIG. 2



INVENTORS.  
OTTO PETER  
HELMUT RECKHARD  
BY

Curtis, Morris & Safford  
ATTORNEYS

1

3,171,816

## FABRICATION OF CARBON BODIES

Otto Peter, Hofheim, Taunus, and Helmut Reckhard, Frankfurt am Main, Germany, assignors to Farbwerke Hoechst Aktiengesellschaft, vormals Meister Lucius & Brüning, Frankfurt am Main, Germany, a corporation of Germany

Filed Nov. 29, 1960, Ser. No. 72,492  
Claims priority, application Germany, Dec. 3, 1959,  
F 29,994

6 Claims. (Cl. 252—510)

The present invention relates to agents for reducing the softening point of binding pitch, as used in the fabrication of carbon bodies.

For the fabrication of carbon bodies the petrol- and/or coal tar pitch coke having a certain gradation of grain sizes and being used as dry material, is mixed with a binding agent, preferably coal tar pitch, and formed in the usual manner. Then the carbon body is baked in a furnace at about 1000° C. and, if necessary, subjected to a graphitization process at temperatures above 2000° C. When baked in the furnace, the binding pitch carbonizes to form a coke skeleton that cements the individual grains of coke and imparts a corresponding strength to the carbon body. Since the strength depends, in general, on the yield of coke of the binding agent, the artificial carbon industries prefer as binding agents pitches having a softening point that is as high as possible. However, there are technological limits with respect to the utilization of pitch since a pitch that has a high softening point requires a higher processing temperature when being mixed and pressed. In order to overcome these difficulties, the softening point of pitches that have a high softening point is reduced to a lower softening point. As agents reducing the softening points of binding pitches there were used hitherto coal tar or higher fractions of coal tar having an oily consistency. However, these known agents have the drawback that the yield of coke of the binding agent, calculated on the binding pitch, remains practically unchanged since the agents themselves do not furnish any coke or only a small portion of coke, i.e. the binding agent, is, so to speak, only fluxed by the substances used for reducing the softening point. This, however, results in a deterioration of the quality of the carbon bodies obtained with respect to their specific weight, strength and volume of voids since, when baking the carbon bodies, a greater quantity of gas escapes than in the case of baking the carbon bodies that do not contain agents for reducing the softening points of the binding pitches. Moreover, it was found that the agents used hitherto only bring about a slight reduction of the softening point due to the partly high viscosity of said agents.

Now we have found that the drawbacks of the known agents reducing the softening points of the binding pitches can be avoided when using for the fabrication of carbon bodies according to the invention organic compounds that are soluble in the binding pitch and contain one or more active double or triple bonds, singly or in admixture with one another, as agents reducing the softening points of the binding pitches.

According to the invention, those organic compounds have proved to be especially advantageous that contain one or several C=C—, C≡C (for example, unsaturated hydrocarbons, vinyl or acetylene derivatives), C=O (for example, ketones, aldehydes, quinones, C=NH (for example imines), C≡N (for example nitriles), C=S (thio compounds, for example xanthates), or N=N— compounds (azo compounds).

When using the proposed compounds as agents that reduce the softening points of the binding pitches, there are obtained, while adding the same amount of agent, not only a greater reduction of the softening point of the

2

binding pitch but simultaneously also a partly considerable increase in the yield of coke of the binding pitch as compared with the use of the formerly applied agents.

FIGS. 1 and 2 of the accompanying drawings represent 5 diagrams illustrating the dependence of the softening point and the yield of coke of a binding pitch on the quantity added of the agents reducing the softening points of the binding pitches as used hitherto and as used according to the invention.

10 In FIG. 1, there are indicated in the ordinate, in °C., the softening points, determined according to Krämer-Sarnow, of a pitch used as a binding agent, and in FIG. 2 the yields of coke of said pitch determined according to Elektrokemisk, calculated on the pitch used, and in 15 the abscissa there is indicated, in percent by weight, the respective addition of the agents reducing the softening points of the binding pitches.

FIG. 1 shows that when using, according to the invention, phthalodinitrile, azobenzene, styrene or phenyl-acetylene as agents reducing the softening points of the 20 binding pitches, the softening points of the binding pitches are reduced in a higher degree than in the case of the tar oils used hitherto, while FIG. 2 distinctly shows that by using the proposed agents the yield of coke of the binding 25 pitch is simultaneously increased appreciably.

In Table 1, there are listed a number of organic compounds that may be used as agents reducing the softening points of the binding pitches according to the invention, 30 said compounds containing one or several active carbon-carbon bonds; in Table 2 there are listed compounds containing one or several active carbon-oxygen bonds, and in Table 3 those compounds containing one or several active carbon-nitrogen bonds. In the second column there is listed the respective addition of the agent reducing 35 the softening points of the binding pitches (in percent by weight), in the third column the softening point determined according to Krämer-Sarnow, and in the fourth column the yield of coke of the binding pitch determined according to Elektrokemisk.

40 The figures given in brackets in the third and fourth columns refer, respectively, to the values of the pure binding pitch without the addition of an agent reducing the softening point of said pitch.

The selectively dehydrogenating effect of the proposed 45 agents reducing the softening points of the binding pitches must especially be stressed, which effect is due to the fact that said agents condense by oxidation only part of the compounds present in the coal tar pitch, for example fluorene-, acenaphthene-, carbazole derivatives and other 50 compounds with relatively easily mobile hydrogen atoms, while another part, for example chrysene, pyrene, etc., is not dehydrogenated. It is, therefore, decisive for the action of the additives according to the invention that, in addition to their solubility in the binding pitch which 55 brings about a reduction of the softening point, their dehydrogenating action, on the one hand, is strong enough to dehydrogenate compounds of coal tar pitch with mobile hydrogen but that, on the other hand, the action is not strong enough to bring about a dehydrogenation at the aromatic nucleus itself. Thanks to this selective dehydrogenation, no change can be ascertained in practice in the properties of the binding coke obtained from the pitch after baking, properties such, for example, as the thermal 60 ratio of expansion, the capability for being graphitized and the hardness, in spite of an increase in the yield of coke of the binding agent. This is of great importance especially for carbon bodies that are to be subjected to a subsequent graphitization process since all condensing 65 agents for increasing the yields of coke proposed hitherto such, for example, as sulfur, metal oxides and metal chlorides, organic nitro- and chlorine compounds, oxygen compounds and compounds that yield oxygen, due to

70

their strong oxidizing action, dehydrogenate the compounds present in the binding pitch to such a degree that the binding coke obtained therefrom has a high coefficient of expansion and a reduced capability for being graphitized. Moreover, when using, for example, nitro compounds and oxygen-yielding substances such, for example, as peroxides, there are formed large amounts of water in the course of the dehydrogenation which, especially in the fabrication of carbon, impairs the structure and, thereby, also the strength of the carbon body.

As compared with the known agents for reducing the softening points of the binding pitches, the compounds according to the present invention possess many advantages, for example, when using the proposed compounds, the softening points of the binding pitches are much more reduced although adding, in each case, the same amount of the agent which amounts to a decrease of the dynamic viscosity since the softening points determined according to Krämer-Sarnow must be regarded as the equiviscosity temperature for the viscosity of about  $10^7$  cp. By reducing the viscosity of the binding pitch, therefore, either the temperature may be decreased when mixing the coal tar pitch coke and the binding agent, or a binding pitch having a higher softening point may be used.

Another advantage of the proposed compounds consists in the increase of the yield of coke of the binding agent which results in an improvement of the properties of the carbon bodies such as an increase of the specific weight and the strength and a lower volume of voids. On the other hand, in spite of the increased yield of coke, no change in the physical properties of the coke of the

however, are not intended to limit the invention thereto, the parts being by weight:

#### Example 1

Twenty kilos of coal tar pitch coke which has, in all examples, the same gradation of grain sizes, i.e.

10 parts—0.75–1.2 mm.

40 parts—0.06–0.75 mm.

50 parts— $<0.06$  mm.

are mixed with 5 to 5.5 kilos of dry pitch A (softening point  $78^{\circ}$  C.) and the agents reducing the softening points of the binding pitches enumerated in the following table (percent by weight, calculated on the weight of the dry pitch used) at  $120^{\circ}$  C. to  $160^{\circ}$  C., and formed in the usual manner on a hydraulic extruder into round electrodes having a diameter of 70 mm., baked in the ring furnace at  $1000^{\circ}$  C. for 3 weeks and subsequently graphitized in the usual manner.

The properties of the graphitized round electrodes are listed in the following Table 4.

For the purpose of comparison, round electrodes having a diameter of 70 mm. obtained from a moist pitch of the same origin (softening point  $57^{\circ}$  C.) are fabricated without the addition of agents reducing the softening points of the binding pitches. The softening points of the pitches used, which were fluxed according to the invention, were determined in special tests in which the agent reducing the softening points of the pitches was introduced into the pitch with agitation.

TABLE 4

|                                                                                             | Softening point, °C. | Yield of coke, <sup>1</sup> percent | Specific weight, kg./l. | Volume of voids, percent | Flexural strength, kg./cm. <sup>2</sup> | Resistance to pressure, kg./cm. <sup>2</sup> |
|---------------------------------------------------------------------------------------------|----------------------|-------------------------------------|-------------------------|--------------------------|-----------------------------------------|----------------------------------------------|
| Dry pitch A                                                                                 | 78                   | 61.1                                | 1.592                   | 22.8                     | 102                                     | 238                                          |
| Dry pitch A+15% of tar                                                                      | 61.5                 | 58.5                                | 1.578                   | 23.1                     | 95                                      | 246                                          |
| Dry pitch A+20% of heavy tar oil                                                            | 56                   | 53                                  | 1.626                   | 22.5                     | 100                                     | 246                                          |
| Dry pitch A+10% of vinyl acetate                                                            | 50                   | 64.2                                | 1.678                   | 19.6                     | 114                                     | 308                                          |
| Dry pitch A+5% of styrene                                                                   | 57                   | 59.9                                | 1.634                   | 20.9                     | 120                                     | 265                                          |
| Dry pitch A+10% of phthalodinitrile                                                         | 59.5                 | 73.0                                | 1.704                   | 17.5                     | 119                                     | 347                                          |
| Dry pitch A+10% of acrylonitrile                                                            | 54                   | 66.4                                | 1.680                   | 19.4                     | 110                                     | 314                                          |
| Soft pitch without the addition of agents reducing the softening point of the binding pitch | 57                   | 54.8                                | 1.589                   | 23.0                     | 97                                      | 205                                          |

<sup>1</sup> Calculated on the pitch and on the agent reducing the softening point of the pitch.

binding agent was observed in practice. This phenomenon is of importance especially in the case of carbon bodies that are to be subjected to a subsequent graphitization process.

The advantages of the compounds according to the invention as agents reducing the softening points of the binding pitches as compared with the compounds used hitherto are illustrated by the following examples which,

Twenty kilos of petrol coke having the same gradation of grain sizes as in Example 1, are mixed at  $120^{\circ}$  to  $160^{\circ}$  C. with 5 to 5.5 kilos of dry pitch (softening points  $79^{\circ}$ ,  $75^{\circ}$ ,  $71.5^{\circ}$  C.) and the agents reducing the softening points of the binding pitches as listed in the following Tables 5 to 7, and formed into round electrodes having a diameter of 70 mm., as described in Example 1.

TABLE 5

|                                                                           | Softening point, °C. | Yield of coke, percent | Specific weight, kg./l. | Volume of voids, percent | Flexural strength, kg./cm. <sup>2</sup> | Resistance to pressure, kg./cm. <sup>2</sup> |
|---------------------------------------------------------------------------|----------------------|------------------------|-------------------------|--------------------------|-----------------------------------------|----------------------------------------------|
| Dry pitch A                                                               | 79                   | 59.1                   | 1.548                   | 25.8                     | 70                                      | 196                                          |
| Dry pitch A+10% of light tar oil                                          | 60                   | 54.2                   | 1.533                   | 25.8                     | 70                                      | 184                                          |
| Dry pitch A+15% of heavy tar oil                                          | 60                   | 50.1                   | 1.507                   | 27.1                     | 58                                      | 162                                          |
| Dry pitch A+15% of tar                                                    | 61                   | 54.0                   | 1.542                   | 25.1                     | 70                                      | 192                                          |
| Dry pitch A+10% of phthalodinitrile                                       | 58                   | 70.3                   | 1.643                   | 21.2                     | 92                                      | 256                                          |
| Dry pitch A+10% of azobenzene                                             | 55                   | 62.3                   | 1.575                   | 23.3                     | 81                                      | 204                                          |
| Soft pitch (without the addition of agents reducing the softening points) | 63.5                 | 51.6                   | 1.517                   | 26.0                     | 70                                      | 169                                          |

TABLE 6

|                                                                          | Softening point, °C. | Yield of coke, percent | Specific weight, kg./l. | Volume of voids, percent | Flexural strength, kg./cm. <sup>2</sup> | Resistance to pressure, kg./cm. <sup>2</sup> |
|--------------------------------------------------------------------------|----------------------|------------------------|-------------------------|--------------------------|-----------------------------------------|----------------------------------------------|
| Dry pitch B                                                              | 75                   | 55.5                   | 1.565                   | 25.9                     | 90                                      | 205                                          |
| Dry pitch B+10% of light tar oil                                         | 57                   | 54.3                   | 1.544                   | 26.7                     | 68                                      | 173                                          |
| Dry pitch B+15% of tar                                                   | 58                   | 56.1                   | 1.559                   | 26.2                     | 69                                      | 178                                          |
| Dry pitch B+10% of phthalodinitrile                                      | 47.5                 | 71.6                   | 1.634                   | 22.4                     | 104                                     | 254                                          |
| Dry pitch B+10% of azobenzene                                            | 49                   | 62.0                   | 1.617                   | 23.3                     | 98                                      | 223                                          |
| Soft pitch (without the addition of agents reducing the softening point) | 60.5                 | 53.5                   | 1.562                   | 26.0                     | 79                                      | 186                                          |

TABLE 7

|                                                                          | Softening point, °C. | Yield of coke, percent | Specific weight, kg./l. | Volume of voids, percent | Flexural strength, kg./cm. <sup>2</sup> | Resistance to pressure, kg./cm. <sup>2</sup> |
|--------------------------------------------------------------------------|----------------------|------------------------|-------------------------|--------------------------|-----------------------------------------|----------------------------------------------|
| Dry pitch C                                                              | 71.5                 | 57.4                   | 1.572                   | 24.4                     | 85                                      | 213                                          |
| Dry pitch C+10% of light tar oil                                         | 54.5                 | 56.0                   | 1.550                   | 25.0                     | 77                                      | 204                                          |
| Dry pitch C+15% of heavy tar oil                                         | 53                   | 55.9                   | 1.545                   | 25.8                     | 69                                      | 210                                          |
| Dry pitch C+10% of azobenzene                                            | 54                   | 57.1                   | 1.574                   | 25.2                     | 87                                      | 230                                          |
| Dry pitch C+10% of phthalodinitrile                                      | 47.5                 | 60.7                   | 1.582                   | 24.1                     | 95                                      | 240                                          |
| Soft pitch (without the addition of agents reducing the softening point) | 48                   | 68.2                   | 1.611                   | 24.1                     | 114                                     | 269                                          |
|                                                                          | 60.5                 | 56.4                   | 1.565                   | 25.6                     | 89                                      | 223                                          |

*Example 3*

Twenty kilos of petrol coke having the same gradation of grain sizes as in Examples 1 and 2 are mixed with approximately 5 to 5.5 kilos of ultra dry pitch (softening point 160° C.) and the agents or mixtures reducing the softening points of the binding pitch as listed in Table 8, and formed into round electrodes having a diameter of 70 mm. according to Example 1.

also a substantial increase in the yield of coke. Moreover, the quality of the carbon body is distinctly improved due to the increase in the specific weight and the strength values as well as on account of the lower volume of voids. The values lie, in all cases, even distinctly above the values of the reference samples obtained with the use of the original dry pitch, although the softening point was decreased considerably.

TABLE 8

|                                                         | Softening point, °C. | Yield of coke, percent | Specific weight, kg./l. | Volume of voids, percent | Flexural strength, kg./cm. <sup>2</sup> | Resistance to pressure, kg./cm. <sup>2</sup> |
|---------------------------------------------------------|----------------------|------------------------|-------------------------|--------------------------|-----------------------------------------|----------------------------------------------|
| Ultra dry pitch+20% of light tar oil                    | 71                   | 67.6                   | 1.590                   | 23.7                     | 106                                     | 238                                          |
| Ultra dry pitch+10% of styrene +10% of phthalodinitrile | 55                   | 80.5                   | 1.645                   | 20.4                     | 115                                     | 306                                          |
| Ultra dry pitch+5% of styrene +15% of phthalodinitrile  | 77                   | 85.2                   | 1.650                   | 17.9                     | 136                                     | 354                                          |

The examples cited distinctly show the superiority of the agents reducing the softening points of the binding pitch as compared with the agents used hitherto. When applying the same amount of additive, there is not only attained a greater decrease in the working temperature but

it has become possible to work up pitches having a very high softening point by using mixtures of the proposed agents reducing the softening points of the binding pitch, 50 the superiority of these substances as compared with the agents used hitherto again manifesting itself.

TABLE 1  
[>C=C< and -C≡C-]

|                                                                                                         | Addition to the binding pitch, percent | Softening point, °C. | Yield of coke, percent |
|---------------------------------------------------------------------------------------------------------|----------------------------------------|----------------------|------------------------|
| Propargyl alcohol CH—C—CH <sub>2</sub> OH                                                               | 10                                     | 49.5 (56)            | 48 (41.5)              |
| Indene →             | 10<br>46                               | 27.5 (57)<br>46 (78) | 46 (42)<br>55 (51)     |
| A cenaphthylene      | 10<br>54                               | 43 (62)<br>54 (81.5) | 50.5 (43.5)<br>57 (50) |
| Dicyclopentadiene →  | 10<br>50                               | 40 (62)<br>50 (81.5) | 48 (43.5)<br>54 (50)   |

7 TABLE 1—Continued

|                                                                                                | Addition to<br>the binding<br>pitch,<br>percent | Softening<br>point, °C. | Yield of<br>coke,<br>percent |
|------------------------------------------------------------------------------------------------|-------------------------------------------------|-------------------------|------------------------------|
| Turpentine oil                                                                                 | 10                                              | 37 (63.5)               | 48 (44.5)                    |
| Divinyl benzene                                                                                | 10                                              | 40.5 (81)               | 56 (51)                      |
| 1,6-dimorpholinyl-hexadiyne-2,4                                                                | 10                                              | 65.5 (82)               | 57 (51)                      |
| N-β-chlorallyl-morpholine                                                                      | 10                                              | 45.5 (79)               | 59 (52)                      |
| Methacrylic acid $\text{CH}_2=\text{C}(\text{CH}_3)-\text{COOH}$                               | 10                                              | 45 (57)                 | 44 (42)                      |
| Crotonic acid $\text{CH}_3-\text{CH}=\text{CH}-\text{COOH}$                                    | 10                                              | 40.5 (56)               | 50 (41.5)                    |
| Vinyl propionate $\text{C}_2\text{H}_5\text{COO}-\text{CH}=\text{CH}_2$                        | 10                                              | 27 (57)                 | 46 (42)                      |
| Dibutyl maleate $\text{C}_4\text{H}_9\text{COO}-\text{CH}=\text{CH}_2\text{COO-C}_4\text{H}_9$ | 10                                              | 27 (56)                 | 43.5 (41.5)                  |
| 1,4-dicyclohexanoyl-diacetylene                                                                | 10                                              | 79 (82)                 | 55.5 (51)                    |
| 2-Butylidene-cyclohexanone-1                                                                   | 10                                              | 43 (79)                 | 57 (52)                      |

TABLE 2  
[ $\triangleright\text{C=O}$ ]

|                                                                                                                                                      | Addition to<br>the binding<br>pitch,<br>percent | Softening<br>point, °C. | Yield of<br>coke,<br>percent |
|------------------------------------------------------------------------------------------------------------------------------------------------------|-------------------------------------------------|-------------------------|------------------------------|
| Acetyl acetone $\text{CH}_3-\text{C}(=\text{O})-\text{CH}_2-\text{C}(=\text{O})-\text{CH}_3$                                                         | 10                                              | 29 (57)                 | 46.5 (42)                    |
| Succinimide $\text{H}_2\text{C}-\text{C}(=\text{O})-\text{NH}-\text{C}(=\text{O})-\text{CH}_2$                                                       | 10                                              | 55 (63.5)               | 47 (43.5)                    |
| Naphthalene dialdehyde $\text{C}_2\text{H}_4\text{Naphthalene}-\text{C}(=\text{O})-\text{CH}_2-\text{C}(=\text{O})-\text{CH}_2-\text{C}_2\text{H}_4$ | 10                                              | 53 (63.5)               | 57 (43.5)                    |
| Benzil $\text{C}_6\text{H}_5-\text{C}(=\text{O})-\text{C}(=\text{O})-\text{C}_6\text{H}_5$                                                           | 10                                              | 44.5 (63.5)             | 50 (43.5)                    |
| Anthraquinone $\text{C}_2\text{H}_2\text{C}_4\text{H}_2\text{O}_2$                                                                                   | 10                                              | 57 (61)                 | 51 (45)                      |

TABLE 2—Continued

|                              | Addition to<br>the binding<br>pitch,<br>percent | Softening<br>point, °C. | Yield of<br>coke,<br>percent |
|------------------------------|-------------------------------------------------|-------------------------|------------------------------|
| Cumarinic acid lactone<br>   | 10                                              | 43 (63.5)               | 47 (43.5)                    |
| 2-allyl-oxyanthraquinone<br> | 10                                              | 56.5 (63.5)             | 55.5 (49.5)                  |
| Phenyl isocyanate<br>        | 10                                              | 52 (56)                 | 44.5 (41.5)                  |

TABLE 3  
[>C=N— or —C≡N]

|                                                                                                                                              | Addition to<br>the binding<br>pitch,<br>percent | Softening<br>point, °C. | Yield of<br>coke,<br>percent |
|----------------------------------------------------------------------------------------------------------------------------------------------|-------------------------------------------------|-------------------------|------------------------------|
| Cyanoacetic acid N≡C—CH <sub>2</sub> —COOH<br>Malonic acid dinitrile N≡C—CH <sub>2</sub> —C≡N                                                | 10<br>10                                        | 54 (57)<br>53 (57)      | 51 (42)<br>51 (42)           |
| Benzonitrile<br>                                                                                                                             | 10                                              | 30.5 (57)               | 49.5 (42)                    |
| Adipic acid nitrile N≡C—CH <sub>2</sub> —CH <sub>2</sub> —CH <sub>2</sub> —CH <sub>2</sub> —C≡N                                              | 10                                              | 31 (63.5)               | 49 (44)                      |
| Phenyl isocyanate<br>                                                                                                                        | 10                                              | 52 (56)                 | 44.5 (41.5)                  |
| Succinodinitrile N≡C—CH <sub>2</sub> —CH <sub>2</sub> —C≡N<br>Benzalaniline C <sub>6</sub> H <sub>5</sub> N=CH—C <sub>6</sub> H <sub>5</sub> | 10<br>10                                        | 55 (78)<br>69 (78)      | 52 (50.5)<br>53.5 (50.5)     |

We claim:

1. A process for the fabrication of carbon bodies which comprises shaping into a body a mixture containing grained coke, a binding pitch and an organic compound for reducing the softening point of the binding pitch, said organic compound being a member selected from the group consisting of vinyl acetate, styrene, phthalodinitrile, acrylonitrile, azobenzene, propargyl alcohol, indene, acenaphthylene, dicyclopentadiene, turpentine oil, divinyl benzene, 1,6-dimorpholinyl-hexadiyne-2,4, N-β-chlorallyl-morpholine, methacrylic acid, crotonic acid, vinyl propionate, dibutyl maleate, 1,4-dicyclohexanoyl - diacetylene, 2 - butyldene-cyclohexanone - 1, acetyl acetone, succinimide, naphthalene dialdehyde, benzil, anthraquinone, cumarinic acid lactone, 2-allyloxyanthraquinone, phenyl isocyanate, cyanoacetic acid, malonic acid dinitrile, benzonitrile, adipic acid nitrile, succinodinitrile and benzalaniline, said compound being present in an amount of from about 2% to about 20% by weight calculated on the weight of the binding pitch; and baking the body at a temperature of about 1000° C.

2. In a method of producing shaped and hardened carbon bodies by admixing granular coke with a binding pitch, shaping the resulting mixture and baking it, the improvement which comprises adding, prior to the shaping step, from about 2% to about 20% by weight, calculated on the weight of binding pitch, of vinyl acetate.

3. In a method of producing shaped and hardened

carbon bodies by admixing granular coke with a binding pitch, shaping the resulting mixture and baking it, the improvement which comprises adding, prior to the shaping step, from about 2% to about 20% by weight, calculated on the weight of binding pitch, of styrene.

4. In a method of producing shaped and hardened carbon bodies by admixing granular coke with a binding pitch, shaping the resulting mixture and baking it, the improvement which comprises adding, prior to the shaping step, from about 2% to about 20% by weight, calculated on the weight of binding pitch, of phthalodinitrile.

5. In a method of producing shaped and hardened carbon bodies by admixing granular coke with a binding pitch, shaping the resulting mixture and baking it, the improvement which comprises adding, prior to the shaping step, from about 2% to about 20% by weight, calculated on the weight of binding pitch, of acrylonitrile.

6. In a method of producing shaped and hardened carbon bodies by admixing granular coke with a binding pitch, shaping the resulting mixture and baking it, the improvement which comprises adding, prior to the shaping step, from about 2% to about 20% by weight, calculated on the weight of binding pitch, of azobenzene.

References Cited in the file of this patent

UNITED STATES PATENTS

2,527,596 Shea et al. \_\_\_\_\_ Oct. 31, 1950  
2,761,848 Bushong et al. \_\_\_\_\_ Sept. 4, 1956